

## UNITED STATES PATENT OFFICE.

FRANK F. COLCORD, OF NEW YORK, N. Y., ASSIGNOR TO UNITED STATES SMELTING, REFINING & MINING COMPANY, OF PORTLAND, MAINE, A CORPORATION OF MAINE.

## ELECTROLYTIC REFINING OF METALS.

No Drawing.

Application filed June 1, 1925. Serial No. 34,222.

The invention relates to the electrodeposition of metals and more particularly to the electrodeposition of zinc.

It is the practice in the electrodeposition of zinc to use so-called addition reagents in the electrolyte and the present invention is based on the discovery of a new reagent of this character which may be used with marked advantage over prior reagents in the electrodeposition of zinc. This reagent is a sulphite liquor concentrate comprising the solid or viscous materials obtained from the waste sulphite liquors produced by treating certain woods with sulphite solutions. The evaporation of these liquors leaves a colloidal substance which may be designated as sulphite lignose. The principal constituents of this substance are or may be lignin sulphuric acid, lignin sulphonic acid, aldehyde sulphonic acids, furfural, and plant sugars. This substance is cheaply made from the waste sulphite liquors produced from the manufacture of paper pulp and is known under the trade names "lignol" and "goulac."

I have discovered that sulphite lignose may be used as an addition reagent in certain electrolytes with remarkably advantageous results. It may be used to replace many of the addition reagents commonly used, weight for weight, and owing to its extremely low price, a substantial economy may be effected. It may be used alone or in partial replacement of some of the commonly used addition reagents effecting not only an economy thereby, but permitting the substitution to take place in an old electrolyte and thus avoid the cost of new electrolyte when changing over to this addition reagent. In many cases it produces a cathode deposit superior to deposits obtained from other addition reagents, increasing thereby the efficiency of the operation and resulting in an important economy in the power consumption. No accumulation in the electrolyte of substances which might finally cause the deposit to form non-adherent and crystalline

deposits has been noticed with this addition reagent, as in the case with some of the prior addition reagents commonly used.

The use of this addition reagent has given particularly excellent results in the electrodeposition of zinc with a sulphuric acid electrolyte. While the composition of the electrolyte can vary considerably without materially affecting the character of the deposit, excellent results have been obtained with an electrolyte which at the start contained 100 grams of zinc as zinc sulphate per liter, and which at the end contained 30 grams of zinc and 100 grams of free sulphuric acid per liter. The common addition reagent in the electrodeposition of zinc has been glue, but complete substitution of this new addition reagent can be effected. In actual practice this addition reagent when used alone is added daily to the electrolyte in the form of a water solution at the rate of one to two pounds of the dry reagent per ton of zinc produced, while if used in conjunction with glue the total quantity of the two reagents added daily is one to two pounds per ton of zinc produced with the glue and the new reagent varying in such proportion as desired. The new reagent alone or in conjunction with other addition reagents produces bright and dense deposits of zinc with sulphuric acid electrolytes.

What is claimed is:

1. That improvement in the electrodeposition of zinc with sulphuric acid electrolytes which consists in the use in the acid electrolyte of sulphite lignose as an addition reagent.
2. That improvement in the electrodeposition of zinc with sulphuric acid electrolytes which consists in the use as an addition reagent in the acid electrolyte of sulphite lignose in conjunction with other addition reagents.

In testimony whereof I have signed my name to this specification.

FRANK F. COLCORD.